

## United States Patent Office

3,345,250

Patented Oct. 3, 1967

1

3,345,250

**BLEACHING PULP WITHOUT DIRECT CHLORINATION BY BLEACHING WITH CHLORINE DIOXIDE**

Amiel W. Brinkley, Jr., Mobile, Ala., and Jack F. Kilborn, Natchez, Miss., assignors to International Paper Company, New York, N.Y., a corporation of New York

No Drawing. Continuation of application Ser. No. 285,578, June 5, 1963. This application June 30, 1966, Ser. No. 562,963

3 Claims. (Cl. 162—78)

The process of this invention is particularly suitable for use upon dissolving grades of cellulosic pulp prepared or "post-treated" in accordance with co-pending U.S. application, Ser. No. 176,489, filed Feb. 23, 1962 as a continuation-in-part of U.S. application 810,877, filed May 4, 1959 and both now abandoned. Indeed, the present application must properly be regarded as a continuation-in-part of Ser. No. 176,489, filed Feb. 23, 1962, and is a continuation of Ser. No. 285,578 filed June 5, 1963, now abandoned.

This invention relates to an improvement in the process of manufacturing a dissolving grade of cellulosic pulp for use in the manufacture of textile or tire grade rayon, cellophane or other cellulosic products manufactured by the viscose process. More specifically, this improvement involves a new method of bleaching dissolving grades of cellulosic pulps which improves the viscose filterability and the rayon strength properties of these pulps. This improved bleaching sequence involves omission of the usual direct chlorination stage, but produces pulps with high brightness and high viscosity by a combination of hypochlorite, caustic extraction and chlorine dioxide stages.

Historically, direct chlorination, which is treatment of the pulp with elemental chlorine gas, has been necessary as a preliminary bleaching stage in order to produce pulps with high brightness without undue degradation of the cellulose. This direct chlorination reacts with the lignin in the unbleached pulp rendering it soluble in caustic and therefore, the chlorination stage is generally followed by a caustic extraction stage to dissolve the chlorinated lignins. Thus, for example, where the lignin content of unbleached dissolving pulps made from softwoods such as southern pine is approximately 3 to 4% when the pre-hydrolyzed kraft cooking process is used and where dissolving pulps cooked in the same manner from hardwoods such as sweetgum or oak, as well as grasses such as bamboo or sugar cane bagasse, have a lignin content of about 1 to 2% before bleaching, the combination of chlorination and caustic extraction normally removes approximately 80% of the lignin present in the unbleached pulp. Following the chlorination and caustic extraction stages, additional bleaching stages are necessary to remove the residual lignin and coloring matter in the pulp to produce high brightness and purity.

As recently as 1953, the bleaching chemicals available to complete the bleaching and purification of pulps degraded the cellulose rather severely at the same time that these chemicals were removing the lignin and coloring matter from the pulp. Hypochlorite or chlorine dioxide under alkaline conditions were generally used. However, in recent years, the use of chlorine dioxide under

2

acid conditions has developed to the point where cellulosic fibers can be bleached to high brightness and purity with very little degradation of the cellulose. The development of corrosion resistant materials and processes for economically generating chlorine dioxide have made the use of this chemical in large quantities possible and economically practical.

It has now been found that cellulosic materials such as pulps from hardwoods or grasses, which have a fairly low lignin content before bleaching, can be bleached fairly economically by a sequence which omits the chlorination stage and instead uses chlorine dioxide or a mild hypochlorite treatment as the first bleaching stage. Not only is such a sequence economically practical, but it also produces pulps which have better viscose filterability and rayon strength stability than pulps bleached by a normal sequence which includes a chlorination stage. This unexpected phenomenon has been proved repeatedly in the laboratory and in mill trials.

It has now also been found that, when the chlorination stage is omitted, it becomes necessary to treat the pulp in the first stage with some type of acid in order to reduce the minerals which otherwise interfere with the bleaching and result in a low pulp brightness. Presumably, the acid conditions that exist in a normal chlorination stage are sufficient to remove these minerals which are primarily iron and manganese, and therefore no acid treatment is required for this type bleaching.

The fact that softwood kraft dissolving pulps have almost twice as much lignin or bleaching chemical demand as similar pulps from hardwoods or grasses and the fact that chlorine dioxide costs twice as much as the equivalent amount of chlorine result in a large cost penalty for bleaching a softwood kraft pulp without chlorination.

Nevertheless, softwood pulps can be bleached in this manner with a view to achieving improved viscose filterability and rayon strength stability compared to similar pulps bleached with the normal sequence involving a chlorination stage.

Again dissolving pulps cooked by other processes such as the sulfite process and which have relatively low lignin contents before bleaching can be bleached readily without a chlorination stage to produce rayon with better viscose filterability and rayon strength properties than a similar pulp bleached with chlorination.

For a clearer understanding of the present invention, reference should be made to attached Tables 1 to 4 which summarize the work done to provide the requisite showing to enable any person skilled in the art to use such invention and to provide a means of comparing the results of such work with the results of other work based on the utilization of chlorine gas as a bleaching agent. Table 2 shows, for instance, that textile grade rayon from bamboo pulp bleached without chlorination had about the same airdry tensile strength, but significantly better tensile strength after ovendrying at 105° C. for 16 hours than did rayon from the same kind of pulp, which was bleached with chlorination. Viscose filterability was also improved by bleaching without chlorination. Again, Tables 3 and 4 show that, within their ambit, bleaching without chlorination significantly improved the airdry tensile strength and elongation as well as the wet tensile strength and elongation.

60

TABLE 1.—BAMBOO DISSOLVING PULP

| Raw material                                                                                                                                                     | Bamboo                            |                                   |
|------------------------------------------------------------------------------------------------------------------------------------------------------------------|-----------------------------------|-----------------------------------|
|                                                                                                                                                                  | Without Chlorination              | With Chlorination                 |
| Type bleaching                                                                                                                                                   |                                   |                                   |
| Permanganate number                                                                                                                                              | 8.4                               | 8.4                               |
| Unbleached viscosity, TAPPI T-230, 1% CED, cp                                                                                                                    | 130<br>AHDEDH <sup>1</sup><br>224 | 130<br>CEHEDH <sup>1</sup><br>223 |
| Bleaching sequence                                                                                                                                               |                                   |                                   |
| Composite number                                                                                                                                                 |                                   |                                   |
| I. Chlorination or Sulfuric Acid (3.0% consistency, 60 minutes):                                                                                                 |                                   |                                   |
| Cl <sub>2</sub> , percent                                                                                                                                        |                                   | 2.45                              |
| H <sub>2</sub> SO <sub>4</sub> , percent                                                                                                                         | 0.80                              |                                   |
| Temperature, °F                                                                                                                                                  | 82                                | 81                                |
| Residual, g.p.l. available Cl <sub>2</sub>                                                                                                                       | 0.10                              |                                   |
| II: Caustic Extraction or Sodium Hypochlorite (120 minutes retention):                                                                                           |                                   |                                   |
| NaOH, percent                                                                                                                                                    | 1.39                              | 1.25                              |
| NaOCl, percent available chlorine                                                                                                                                | 3.72                              |                                   |
| Temperature, °F                                                                                                                                                  | 111                               | 160                               |
| Consistency, percent                                                                                                                                             | 12.0                              | 10.0                              |
| pH off                                                                                                                                                           | 10.3                              | 10.3                              |
| Residual, g.p.l. available Cl <sub>2</sub>                                                                                                                       | 0.20                              |                                   |
| Residual NaOH, g.p.l.                                                                                                                                            |                                   | 0.37                              |
| Viscosity, TAPPI T-230, 1% CED, cp                                                                                                                               | 28                                | 50                                |
| III. Sodium Hypochlorite or Chlorine Dioxide:                                                                                                                    |                                   |                                   |
| NaOCl, percent available chlorine                                                                                                                                | 1.10                              |                                   |
| NaOH, percent                                                                                                                                                    | 0.43                              |                                   |
| ClO <sub>2</sub> , percent                                                                                                                                       | 0.62                              |                                   |
| Temperature, °F                                                                                                                                                  | 160                               | 125                               |
| Consistency, percent                                                                                                                                             | 10.0                              | 12.0                              |
| Retention, minutes                                                                                                                                               | 180                               | 120                               |
| pH off                                                                                                                                                           | 4.2                               | 10.2                              |
| Residual, g.p.l. available Cl <sub>2</sub>                                                                                                                       | 0.10                              | 0.14                              |
| Viscosity, TAPPI T-230, 1% CED, cp                                                                                                                               | 27.5                              | 27                                |
| IV. Caustic Extraction (10.0% consistency, 120 minutes, 160° F.):                                                                                                |                                   |                                   |
| NaOH, percent                                                                                                                                                    | 0.50                              | 0.25                              |
| pH off                                                                                                                                                           | 11.2                              | 11.4                              |
| Residual NaOH, g.p.l.                                                                                                                                            | 0.33                              | 0.21                              |
| Viscosity, TAPPI T-230, 1% CED, cp                                                                                                                               | 26.5                              | 25.0                              |
| V. Chlorine Dioxide (10.0% consistency):                                                                                                                         |                                   |                                   |
| ClO <sub>2</sub> , percent                                                                                                                                       | 0.20                              | 0.25                              |
| Temperature, °F                                                                                                                                                  | 160                               | 160                               |
| Retention, minutes                                                                                                                                               | 180                               | 180                               |
| pH off                                                                                                                                                           | 5.1                               | 4.3                               |
| Residual, g.p.l. available Cl <sub>2</sub>                                                                                                                       | 0.13                              | 0.10                              |
| Viscosity, TAPPI T-230, 1% CED, cp                                                                                                                               | 26.2                              | 24.8                              |
| Sodium Hypochlorite <sup>2</sup> (one or more stages at 6.5% consistency for 3 hours at temperature and chemical concentration necessary for desired viscosity): |                                   |                                   |
| Final G.E. brightness, TAPPI                                                                                                                                     | 91.1                              | 91.0                              |
| Final viscosity, TAPPI T-230, 1% CED, cp                                                                                                                         | 16.8                              | 17.8                              |
| Total Chemicals (corrected for excess chlorine and sodium hypochlorite residual):                                                                                |                                   |                                   |
| Cl <sub>2</sub> , percent                                                                                                                                        | 4.05                              | 3.63                              |
| NaOH, percent                                                                                                                                                    | 7.21                              | 3.40                              |
| ClO <sub>2</sub> , percent                                                                                                                                       | 0.82                              | 0.25                              |
| H <sub>2</sub> SO <sub>4</sub> , percent                                                                                                                         | 0.80                              |                                   |
| SO <sub>2</sub> , percent                                                                                                                                        | 1.89                              | 1.50                              |

<sup>1</sup> A—sulfuric acid pretreatment, C—chlorination, E—caustic extraction, D—chlorine dioxide, H—sodium hypochlorite.

<sup>2</sup> After the hypochlorite stages, these pulps were centri-cleaned and given two sulfur dioxide treatments for 30 minutes each, 5.0% consistency, 5.0 to 3.0 pH, and 125 to 130° F. before making viscose handsheets.

TABLE 2.—BAMBOO DISSOLVING PULP

| Raw material                 | Bamboo                               |                              |
|------------------------------|--------------------------------------|------------------------------|
|                              | Without Chlorination                 | With Chlorination            |
| 5                            |                                      |                              |
| Type bleaching               |                                      |                              |
| Composite number             | 10                                   |                              |
| Bleaching sequence           |                                      |                              |
| CO-224<br>AHDED <sup>1</sup> |                                      | CO-223<br>CEHED <sup>1</sup> |
| Viscose Solution Quality     |                                      |                              |
| 15                           | Aging temperature, °C                | 25.0                         |
|                              | Aging time, hr. (40 visc.)           | 25                           |
|                              | Temperature requirement (40 visc.)   | 23.0                         |
|                              | Spinning viscosity (36 hr.)          | 35.8                         |
|                              | Filterability, Canton, percent       | 86                           |
|                              | Filterability, nylon, percent        | 75                           |
|                              | Filterability, nylon plugging volume | 86                           |
| 20                           |                                      |                              |
| Rayon Quality                |                                      |                              |
| 25                           | Denier, g.                           | 173.0                        |
|                              | Airdry:                              |                              |
|                              | Tensile, g./denier cond.             | 2.41                         |
|                              | Elongation, percent cond.            | 17.7                         |
|                              | Tensile, g./denier wet               | 1.09                         |
|                              | Elongation, percent wet              | 34.5                         |
| 30                           | Ovendry reconditioned:               |                              |
|                              | Tensile, g./denier cond.             | 2.32                         |
|                              | Elongation, percent cond.            | 16.2                         |
|                              | Tensile, g./denier wet               | 1.03                         |
|                              | Elongation, percent wet              | 31.3                         |
|                              | Heat loss, percent                   | 5.0                          |
|                              | Rayon brightness, desulfured         | 71.6                         |
|                              | Rayon color, desulfured              | 88.2                         |
| 35                           |                                      |                              |
| Physical Properties          |                                      |                              |
| 40                           | Basis weight, lb./1,000 sq. ft.      | 143.4                        |
|                              | Apparent density, g./cc.             | 0.72                         |
|                              | Brightness, percent G.E.             | 91.1                         |
|                              | Fines, percent (100 mesh)            | 21.3                         |
|                              | Dirt, specks/720 sq. in.             | 878                          |
| 45                           |                                      |                              |
| Chemical Analyses            |                                      |                              |
| 50                           | Pulp visc., TAPPI T-230, 1% CED, cp  | 16.8                         |
|                              | Alpha cellulose, percent             | 93.3                         |
|                              | Beta cellulose, percent              | 5.4                          |
|                              | Gamma cellulose, percent             | 1.3                          |
|                              | Ash, percent                         | 0.044                        |
|                              | Pentosans, percent                   | 3.7                          |
|                              | Resins, percent                      | 0.082                        |
|                              | Fe, p.p.m.                           | 20                           |
|                              | Si, p.p.m.                           | 46                           |
|                              | Cu, p.p.m.                           | 7.1                          |
|                              | Mn, p.p.m.                           | 0.4                          |
|                              | 7.14% NaOH solubility                | 10.6                         |
|                              | Copper number                        | 0.60                         |

<sup>1</sup> A—sulfuric acid pretreatment, C—chlorination, E—caustic extraction, D—chlorine dioxide, H—sodium hypochlorite.

TABLE 3.—HARDWOOD DISSOLVING PULPS—BLEACHING

| Bleaching sequence                                               | C <sub>2</sub> EHDDED <sup>1</sup> |           | A <sub>2</sub> EHDDED <sup>1</sup> |           |
|------------------------------------------------------------------|------------------------------------|-----------|------------------------------------|-----------|
|                                                                  | Mixed Hardwoods                    | Sweetgum  | Mixed Hardwoods                    | Sweetgum  |
| Type pulp                                                        |                                    |           |                                    |           |
| Permanganate number                                              | 5.6                                | 4.3       | 5.6                                | 4.3       |
| Viscosity, TAPPI T-230, 1% CED, cp                               | 187                                | 158       | 187                                | 158       |
| Bleach composite number                                          | 245                                | 248       | 247                                | 246       |
| I. Sulfuric Acid or Chlorination (3.0% consistency, 60 minutes): |                                    |           |                                    |           |
| Cl <sub>2</sub> , percent                                        | 1.30                               | 0.75      | 0.40                               | 0.40      |
| ClO <sub>2</sub> , percent                                       | 0.10                               | 0.10      | 0.86                               | 0.79      |
| H <sub>2</sub> SO <sub>4</sub> , percent                         |                                    |           | 2.8                                | 2.8       |
| pH adjusted to                                                   |                                    |           | 100                                | 100       |
| Temperature, °F                                                  | 80                                 | 79        | 2.7                                | 2.7       |
| pH off                                                           | 0.09/0.06                          | 0.03/0.01 | 0.03/0.01                          | 0.02/0.01 |

TABLE 3—Continued

| Bleaching sequence                                                                                                                                         | C <sub>b</sub> EHDED <sup>1</sup> |          | A <sub>b</sub> EHDED <sup>1</sup> |          |
|------------------------------------------------------------------------------------------------------------------------------------------------------------|-----------------------------------|----------|-----------------------------------|----------|
|                                                                                                                                                            | Mixed Hardwoods                   | Sweetgum | Mixed Hardwoods                   | Sweetgum |
| Type pulp                                                                                                                                                  |                                   |          |                                   |          |
| Permanganate number                                                                                                                                        | 5.6                               | 4.3      | 5.6                               | 4.3      |
| Viscosity, TAPPI T-230, 1% CED, cp                                                                                                                         | 187                               | 158      | 187                               | 158      |
| Bleach composite number                                                                                                                                    | 245                               | 248      | 247                               | 246      |
| II. Caustic Extraction (10.0% consistency, 120 minutes):                                                                                                   |                                   |          |                                   |          |
| NaOH, percent                                                                                                                                              | 0.54                              | 0.40     | 0.42                              | 0.32     |
| Temperature, °F                                                                                                                                            | 160                               | 130      | 160                               | 130      |
| pH on                                                                                                                                                      | 11.4                              | 11.2     | 11.4                              | 11.3     |
| pH off                                                                                                                                                     | 9.8                               | 10.2     | 10.6                              | 10.4     |
| Residual, g.p.l. NaOH                                                                                                                                      | 0.17                              | 0.08     | 0.18                              | 0.09     |
| Viscosity, TAPPI T-230, 1% CED, cp                                                                                                                         | 141                               | 122      | 163                               | 140      |
| III. Sodium Hypochlorite (10.0% consistency, 120 minutes):                                                                                                 |                                   |          |                                   |          |
| NaOCl, percent available Cl <sub>2</sub>                                                                                                                   | 0.20                              |          | 0.30                              |          |
| NaOH, percent                                                                                                                                              | 0.08                              |          | 0.09                              |          |
| Temperature, °F                                                                                                                                            | 90                                |          | 90                                |          |
| pH off                                                                                                                                                     | 10.6                              |          | 10.6                              |          |
| Residual, g.p.l. available Cl <sub>2</sub>                                                                                                                 | 0.06                              |          | 0.12                              |          |
| G.E. brightness, heatdry                                                                                                                                   | 74                                |          | 72                                |          |
| Viscosity, TAPPI T-230, 1% CED, cp                                                                                                                         | 134                               |          | 149                               |          |
| IV. Chlorine Dioxide (10.0% consistency, 180 minutes, 140° F.):                                                                                            |                                   |          |                                   |          |
| ClO <sub>2</sub> , percent                                                                                                                                 | 0.26                              | 0.40     | 0.42                              | 0.49     |
| NaOH, percent                                                                                                                                              |                                   | 0.05     |                                   | 0.08     |
| pH off                                                                                                                                                     | 3.6                               | 3.0      | 3.0                               | 3.0      |
| Residual, g.p.l. available Cl <sub>2</sub>                                                                                                                 | 0.16                              | 0.13     | 0.18                              | 0.13     |
| NaOH for neutralization, percent                                                                                                                           | 0.09                              | 0.16     | 0.15                              | 0.15     |
| pH after neutralization                                                                                                                                    | 8.7                               | 7.7      | 7.6                               | 8.0      |
| G.E. brightness, heatdry                                                                                                                                   | 84                                | 82       | 83                                | 82       |
| Viscosity, TAPPI T-230, 1% CED, cp                                                                                                                         | 126                               | 111      | 131                               | 124      |
| V. Caustic Extraction (10.0% consistency, 120 minutes, 140° F.):                                                                                           |                                   |          |                                   |          |
| NaOH, percent                                                                                                                                              | 0.22                              | 0.18     | 0.20                              | 0.22     |
| pH off                                                                                                                                                     | 10.9                              | 10.8     | 11.0                              | 10.9     |
| Residual, g.p.l. NaOH                                                                                                                                      | 0.16                              | 0.14     | 0.16                              | 0.16     |
| Viscosity, TAPPI T-230, 1% CED, cp                                                                                                                         | 120                               | 108      | 121                               | 116      |
| VI. Chlorine Dioxide (10.0% consistency, 180 minutes, 140° F.):                                                                                            |                                   |          |                                   |          |
| ClO <sub>2</sub> , percent                                                                                                                                 | 0.20                              | 0.20     | 0.21                              | 0.20     |
| pH off                                                                                                                                                     | 4.4                               | 4.3      | 4.3                               | 4.2      |
| Residual, g.p.l. available Cl <sub>2</sub>                                                                                                                 | 0.19                              | 0.15     | 0.18                              | 0.16     |
| NaOH for neutralization, percent                                                                                                                           | 0.06                              | 0.05     | 0.06                              | 0.05     |
| pH after neutralization                                                                                                                                    | 8.4                               | 8.2      | 8.0                               | 8.1      |
| G.E. brightness, heatdry                                                                                                                                   | 89                                | 87       | 88                                | 88       |
| Viscosity, TAPPI T-230, 1% CED, cp                                                                                                                         | 111                               | 103      | 116                               | 112      |
| VII. Sodium Hypochlorite (one or more stages at 6.5% consistency for 3 hours at temperatures and chemical concentrations necessary for desired viscosity): |                                   |          |                                   |          |
| Final G.E. brightness, TAPPI <sup>2</sup>                                                                                                                  | 89.4                              | 88.4     | 88.7                              | 87.4     |
| Final Viscosity, TAPPI T-230, 1% CED, cp                                                                                                                   | 100                               | 100      | 101                               | 102      |
| Total Chemicals (corrected for excess chlorine and sodium hypochlorite residual):                                                                          |                                   |          |                                   |          |
| Cl <sub>2</sub> , percent                                                                                                                                  | 1.42                              | 0.75     | 0.23                              |          |
| NaOH, percent                                                                                                                                              | 1.21                              | 0.84     | 1.22                              | 0.82     |
| ClO <sub>2</sub> , percent                                                                                                                                 | 0.56                              | 0.70     | 1.02                              | 1.09     |
| H <sub>2</sub> SO <sub>4</sub> , percent                                                                                                                   |                                   |          | 0.85                              | 0.79     |
| SO <sub>2</sub> , percent                                                                                                                                  | 0.75                              | 0.68     | 0.64                              | 1.00     |

<sup>1</sup> C<sub>b</sub>—chlorination with chlorine dioxide added, A<sub>b</sub>—sulfuric acid with chlorine dioxide added, H—sodium hypochlorite, D—chlorine dioxide, E—caustic extraction.

<sup>2</sup> This pulp was centri-cleaned and given 2 sulfur dioxide treatments for 30 min. each at 5.0% consistency, 2.0 to 2.5 pH, and 125 to 130° F. before making viscose handsheets.

TABLE 4.—HARDWOOD DISSOLVING PULPS

| Type pulp                          | Mixed Hardwoods                             | 100% Sweetgum                               | Mixed Hardwoods                             | 100% Sweetgum                               |
|------------------------------------|---------------------------------------------|---------------------------------------------|---------------------------------------------|---------------------------------------------|
|                                    |                                             |                                             |                                             |                                             |
| Sample number                      |                                             |                                             |                                             |                                             |
| Laboratory bleaching               | CO-245<br>C <sub>b</sub> EHDED <sup>1</sup> | CO-248<br>C <sub>b</sub> EHDED <sup>1</sup> | CO-247<br>A <sub>b</sub> EHDED <sup>1</sup> | CO-246<br>A <sub>b</sub> EHDED <sup>1</sup> |
| Viscose Solution Quality           |                                             |                                             |                                             |                                             |
| Aging temperature, °C              | 26.2                                        | 27                                          | 27.8                                        | 26.2                                        |
| Aging time, hr. (40 visc.)         | 73                                          | 73                                          | 73                                          | 73                                          |
| Temperature requirement (40 visc.) | 25.6                                        | 25.8                                        | 28.2                                        | 26.0                                        |
| Spinning viscosity (36 hr.)        | 35.3                                        | 32.6                                        | 43.4                                        | 38.3                                        |
| Rayon Quality                      |                                             |                                             |                                             |                                             |
| Denier, g.                         | 173.6                                       | 175.2                                       | 174.2                                       | 173.8                                       |
| Tensile, g./denier cond. (Airdry)  | 4.00                                        | 4.34                                        | 4.32                                        | 4.47                                        |
| Elongation, percent cond.          | 9.2                                         | 10.2                                        | 10.0                                        | 10.7                                        |
| Tensile, g./denier wet             | 2.52                                        | 2.80                                        | 2.77                                        | 2.84                                        |
| Elongation, percent wet            | 16.6                                        | 18.0                                        | 17.2                                        | 18.4                                        |
| Tensile, loop, g./denier (Airdry)  | 2.38                                        | 2.49                                        | 2.48                                        | 2.51                                        |
| Tensile, knot, g./denier           | 2.07                                        | 2.09                                        | 2.07                                        | 2.08                                        |
| Elongation, loop, percent          | 5.7                                         | 6.0                                         | 5.8                                         | 5.5                                         |
| Elongation, knot, percent          | 4.9                                         | 5.1                                         | 4.6                                         | 4.4                                         |

See footnotes at end of tables.

TABLE 4.—Continued

| Type pulp                           | Mixed Hardwoods        | 100% Sweetgum          | Mixed Hardwoods        | 100% Sweetgum          |
|-------------------------------------|------------------------|------------------------|------------------------|------------------------|
| Sample number                       | CO-245                 | CO-248                 | CO-247                 | CO-246                 |
| Laboratory bleaching                |                        |                        |                        |                        |
|                                     | C <sub>b</sub> EHDED 1 | C <sub>b</sub> EHDED 1 | A <sub>b</sub> EHDED 1 | A <sub>b</sub> EHDED 1 |
| Physical Properties                 |                        |                        |                        |                        |
| Basis weight, lb./1,000 sq. ft.     | 140                    | 142                    | 140                    | 140                    |
| Apparent density, g./cc.            | 0.73                   | 0.73                   | 0.73                   | 0.73                   |
| Brightness, percent G.E.            | 89.4                   | 88.4                   | 88.7                   | 87.4                   |
| Fines, percent (100 mesh)           | 21.1                   | 11.4                   | 21.8                   | 12.0                   |
| Dirt, specks/720 sq. in.            | 500                    | 580                    | 526                    | 414                    |
| Chemical Analyses                   |                        |                        |                        |                        |
| Viscosity, TAPPI T-230, 1% CED, cp. | 100                    | 100                    | 101                    | 102                    |
| Alpha cellulose, percent            | 95.0                   | 95.4                   | 95.2                   | 95.3                   |
| Ash, percent                        | 0.03                   | 0.02                   | 0.03                   | 0.03                   |
| Pentosans, percent                  | 3.6                    | 3.3                    | 3.5                    | 3.2                    |
| Resins, percent                     | 0.076                  | 0.047                  | 0.064                  | 0.044                  |
| 7.14% NaOH solubility               | 6.03                   | 5.39                   | 5.97                   | 5.09                   |
| Copper number                       | 0.32                   | 0.24                   | 0.18                   | 0.16                   |

<sup>1</sup> C<sub>b</sub>—chlorination with chlorine dioxide added, A<sub>b</sub>—sulfuric acid with chlorine dioxide added, H—sodium hypochlorite, D—chlorine dioxide, E—caustic extraction.

What is claimed is:

1. In a process of preparing wood pulp by subjecting it to a sequence of bleaching and caustic extraction steps without direct chlorination, the step of bleaching the pulp first with chlorine dioxide under acid conditions produced by the addition of an acid to the pulp and then with at least one hypochlorite.
2. In a process of preparing cellulosic pulp by subjecting it to a sequence of bleaching and caustic extraction steps without direct chlorination, the step of bleaching the pulp first with chlorine dioxide under acid conditions produced by the addition of an acid to the pulp.

3. Dissolving grade cellulosic pulp made in accordance with claim 2.

References Cited

UNITED STATES PATENTS

|           |         |          |        |
|-----------|---------|----------|--------|
| 2,494,542 | 1/1950  | Casciani | 162—78 |
| 2,513,788 | 7/1950  | Day      | 162—89 |
| 2,587,064 | 2/1952  | Rapson   | 162—88 |
| 3,020,196 | 2/1962  | Schuber  | 162—78 |
| 3,061,504 | 10/1962 | Mutton   | 162—89 |

DONALL H. SYLVESTER, Primary Examiner.

HOWARD R. CAINE, Examiner.